# EUROPEAN PATENT SPECIFICATION

(11) **EP 0 243 453 B1**
(45) Date of publication and mention of the grant of the patent: **18.07.1990**
(21) Application number: 86906575.5
(22) Date of filing: 06.10.1986
(51) Int. Cl.: B22D 11/06

(54) **DIRECT STRIP CASTING ON GROOVED WHEELS**
BANDSTRANGGIESSEN AUF MIT RILLEN VERSEHENEN GIESSROLLEN
BANDE DE METAL COULEE DIRECTEMENT SUR DES CYLINDRES RAINURES

(30) Priority: 11.10.1985 US 786789
(43) Date of publication of application: 04.11.1987
(73) Proprietor: BATTELLE MEMORIAL INSTITUTE, Columbus Ohio 43201-2693 (US)
(72) Inventor: BARTLETT, Edwin, S., Worthington, OH 43085 (US); MARINGER, Robert, E., Worthington, OH 43085 (US); RAYMENT, Judith, J., Columbus, OH 43201 (US)
(74) Representative: Altenburg, Udo, Dipl.-Phys.
(86) International application number: US8602125
(87) International publication number: WO8702284

(56) References cited:
- FR-A- 1 364 717
- US-A- 4 088 295
- US-A- 4 250 950
- Patent Abstracts of Japan, vol. 7, no. 173, (M-232) (1318) 30 July 1983 & JP, A, 5877748 ( MITSUBISHI JUKOGYO K.K. ) 11 May 1983, see the whole abstract

## Description

### Background of the Invention

The invention relates to a novel method for making metal strip or sheet directly from a molten mass of the metal. From prior patents issued to King (U.S. 3,522,836, U.S. 3,605,863) and others, it is known how to make strip in this manner. King discloses a method whereby a layer of the liquid metal is deposited onto the smooth, outer, cylindrical surface of a chilled roller by a so-called melt drag process. In the melt drag process the moving substrate passes through a meniscus of liquid metal delivered by an orifice and drags the metal from the orifice. The layer quickly solidifies on the chill surface and is removed as a strip.

By the above melt drag method or, so far as we know, by other methods not utilizing an orifice for delivery, the surface of metal strip formed by rapidly chilling a molten metal layer on a smooth substrate may contain various casting defects. These defects are generally a vestige of poor (thermal) contact regions of the liquid metal with the substrate. The poor contact results in slower solidification of metal than in adjacent regions of good contact.

A patent to Buxmann, et al. (U.S. 4,250,950) discloses a metal mold with projections for controlling the rate of metal solidification, but apparently not for improving surface finish as proposed herein.

French Patent 1,364,717 teaches a method for continuous casting of thick metal blanks, in an endless mold. It is somewhat unclear from the disclosure, but at least one and possibly both of the casting surfaces of the mold are rough, for example, they are grooved. It is clear from the disclosure and the continuous casting art that lubrication and release agents are used on the mold and that only thick strip can be formed in this manner. In this way, the disclosed continuous casting method is substantially different than the present process wherein thin strip (less than 10 mm) is made and wherein it must be temporarily bonded to a free casting surface for proper heat transfer.

Other methods exist for producing strip which replicates the surface of the drum (see U.S. 3,561,636 and U.S. 4,212,343, for example). Such methods are not relevant to the present invention because the present method produces smooth metal strip which preferably does not replicate the drum. A rather smooth finish is desired so that the strip may be formed and used as cast (such as for roof gutters, for example) or may be further formed into useful shapes with only a minimum of cold rolling.

The EP-A-147 912, upon which the preamble of claim 1 is based, discloses a method for making strip and fiber from molten mass of metal whereby a layer of the liquid metal is deposited onto a cylindrical surface of a chilled roll. This cylindrical surface may be smooth or grooved with sharp ridges. The chilled roll with smooth surface is specifically used for making strip and this document never says we can make strip on the grooved surface. In any case the grooved surface with sharp ridges disclosed by this document would not be able to give the best surface conditions on the upper surface of the strip.

### Summary of the Invention

The object of the present invention is to improve the surface quality (reduce surface defects) in metal strip formed on a chill surface directly from the melt.

For doing this, an object of this invention relates to a method for casting commercial quality metal sheet of thickness less than about 10 mm according to claim 1.

Preferably the grooves are cut with an included angle of between about 30 and 60 degrees and a depth of about 0.025―0.25 mm. The land region between grooves may vary from 0.025-1.00 mm in width and the ratio of land width to the groove width is preferably greater than 0.15 and more preferably between about 0.5 and 1.5.

Brushing of the chill roll between castings is desirable to clean the casting surface.

Description of the Drawings
Figs. 1 and 2 show a schematic elevation and plan view, respectively, of one tundish and drum assembly for casting metal strip.
Fig. 3 shows two cross-sectional views of land and groove geometries which may be used to cast improved strip according to the invention.
Fig. 4 is a representation of the liquid metal behavior at the surface in contact with the grooved drum.

### Description of the Preferred Embodiments

Figs. 1 and 2 show schematic views of one tundish and chilled roll or drum assembly for practicing the invention. The cylindrical drum 2 is mounted for rotation relative to the tundish 1 and is conventionally water cooled (not shown). The tundish 1 has a contour matching the roller surface at one end and is spaced from the drum 2 such that the liquid metal 10 will not spill during rotation of the drum. Weir 4 smooths out the flow of liquid metal which is made-up by pouring into the tundish at the opposite end from the wheel. Dam 3 forms a pouring chamber with the tundish back wall. Dam 3 and weir 4 also control the melt level 6 and 7 respectively. Weir 5 may be used to control the melt level 8 (the metalostatic head height) and also to control the contact length 9 of the melt with the drum. This contact length is important for controlling the thickness of the strip 11. The weir 5 may alternatively be closely spaced from the drum surface to meter the liquid metal to the surface, i.e. serving as an orifice. Liquid metal 10 contacts the cooled drum and solidifies to the solid strip 11 before removal from the drum.

Typically, the bottom of the tundish approaches the drum at a point about 30° from horizontal, but this point of approach may vary substantially depending on the drum diameter, casting speed and desired strip thickness. The gap between the drum and the tundish may be on the order of 0.15-1.00 mm and the melt contact length with the drum on the order of 4-120 mm. Parameters are preferably adjusted to cast strip less than 10 mm and more preferably less than 1 mm in thickness.

Apparatus including that shown in Fig. 1 have been used in the past for casting metal on a smooth, cylindrical drum surface (for example, a machined surface ground through 600-grit sanding paper). Unfortunately, when metal such as aluminum, copper or steel alloys are cast on smooth wheels, surface defects may arise. These defects are visually perceived in the strip surface as either points, lines or networks of discoloration, texture, relief and/or cracking depending on the severity. The defects appear to be related to areas of poor contact of the liquid metal with the drum surface causing slower solidification of such areas relative to adjacent areas. This differential solidification appears to permanently define a defect region in the solidified strip which is a vestige of the poor contact.

The term "dimple" is used to mean a shallow defect area of 1-2 mm in diameter having a matte surface compared to the otherwise reflective appearance of the strip surface. The dimple is a common defect which the present invention may reduce. The linear defects typically form an irregular mosaic pattern onf depressions which may be the site of cracking. As a result of the slow solidification, bottom surface dimples may result in top surface craters and bottom surface linear depressions result in top surface valleys. Both result in variations in nucleation and grain growth in the regions.

It has been found that these defects can be reduced substantially and both the upper and lower surfaces of the strip can be made smoother by casting on a drum with circumferential grooves in the casting surface. Helical (threaded) or straight-machined grooves are equally acceptable so long as the grooves are substantially circumferential and closely spaced. The rapid wheel speeds preclude surface grooves which are not substantially circumferential because of turbulence in a liquid metal. Grooving results in what is known as a land-and-groove surface having alternating grooves separated by raised land regions.

Fig. 3 shows common grooving which is useful in the invention. In Fig. 3(a) a simple "V" shaped groove 32 has been uniformly machined in the surface of a drum 31 (shown in cutaway). The land regions 33 have a minimum width of 0.025 mm in this grooving. In Fig. 3(b) the land regions 33 have a maximum width ω separating grooves 32. Frequently, the machining process results in a variable pattern of lands according to Fig. 3a and 3b which may also be useful but is not preferred. Extended use and cleaning of the drum may round the edges and flatten the lands.

It has been found that the drum surface should have a groove frequency of about 8-35 grooves/ centimeter measured axially along the surface of the drum from edge 34 to edge 35 in Fig. 3(a). The grooves need not be "V"-shaped but preferably have an average depth of about 0.025-0.25 millimeters. If they are "V"-shaped, the included angle formed by the walls is preferably about 30-60°. The land regions have an average width of about 0.025-1.00 millimeters. Preferably the ratio of average land width to average groove width is about 0.5-1.5, but patterns outside of this range are useful. Generally, only the high land to groove ratio is not particularly useful in producing significant improvement in strip quality as the drum surface approaches the prior art continuous (ungrooved) condition. The grooving need not be uniform but is preferably so.

Delivery of the molten metal at reasonable pressure to the high frequency grooving results in a pattern in which the liquid metal does not completely fill the grooves. Fig. 4 shows a condition of the liquid metal 43 immediately after deposit. The lower surface of the metal is depressed (at 46) into grooves 41 in the drum 40. The surface tension of the liquid may cause the liquid metal to be raised over the land regions 42 between depressions but other pressures may depress the liquid in the groove. Upon solidification the depressions 46 remain in the strip. Except in very thin metal strip and large spacing of grooves, the undulation in the lower surface caused by the grooves is not replicated in the upper surface of the strip. The actual shape of the grooving is not replicated in either the lower or upper surface. However, the upper surface is affected by the lower surface because solidification propagates from the bottom to the top, unlike mold casting process where solidification fronts begin from each mold surface.

After delivery, metal actually adheres to the outer casting surface. We believe this is an atomic bond between the metal and the chill surface and that it is necessary for practicing the present process. The adhesion results in the rapid heat transfer necessary to solidify the strip with the desired microstructure and the consequent shrinkage which causes the strip to break free of the chill surface to be collected. Thus must all take place in a very short time at wheel speeds on the order of 100-1000 cm/sec. Brushing of the drum surface is extremely desirable to keep the drum surface clear of oxides and other impurities which would prevent the necessary bonding.

Such is not the case with continuous casting arts such as disclosed in French Patent 1,364,177. In continuous casting, the object is to cast into a mold, not on a free surface. This necessary limits the product to rather thick blanks (for example, greater than 20 mm) and slow casting speeds. Lubricants and release agents must be used to avoid bonding of metal to the mold. Solidification also takes place from both sides of the mold, causing a layered microstructure and the possibility of internal shrinkage void. Rates of heat transfer are at least an order of magnitude less than for the present rapid solidification process.

The casting drum is preferably water cooled. It may be made of any convenient metal which will withstand the conditions, in particular, the temperature of the molten metal. For example, copper, copper- chromium, steel or aluminum alloy drums may be used selectively for casting aluminum, copper and steel. The grooves may be introduced, for example, by machining or, when the metal is soft enough, by roll threading or embossing. Preferably, a cloth or wire wiper is used with the drum for keeping the grooves clean during use.

Sticking (not the necessary temporary bonding) may be more frequent than with a smooth wheel if the grooves are rough. This can be caused by over-aggressive redressing or wiping of the drum surface causing burrs to form on the land edges. Too high a pressure on the liquid metal during casting on such rough surfaces forces the metal too deeply into the grooves where the metal can solidify and stick on the burrs after the solidification and shrinkage of the strip.

Drum speeds during the casting operation are on the order of 100-1000 cm/sec. Lower speeds can be used to produce thicker strip but, as with any casting process, this would generally result in lower productivity. At the upper end of the stated range and above, the cast strip tends to become thinner as the metal contact time is decreased. Depending on the groove size, this can result in replication of the groove- induced undulation in the upper surface of the strip. For some uses this is not detrimental. Drum size (width and diameter) does not appear to be critical so long as effective cooling can be accomplished and metal can be delivered at the proper rate from the tundish.

### Examples of the Preferred Embodiments

So far as we know, strip directly cast on a cooled drum by other apparatus and methods may benefit from the grooving of the drum according to the invention. However, our experimental trials have been made on smooth and grooved drums using, primarily, the apparatus as shown in Figs. 1 and 2. The drums were made with either copper, copper-1 % chromium alloy, steel or aluminum alloy. Metals cast were aluminum alloy 3105 (nominally AI-0.5% Mg-0.5% Mn), OFHC Copper and low-carbon steel (nominally Fe-0.35% Mn 0.05% C). The cast strip is preferably crystalline with a thickness of greater than 0.25 mm.

"V"-shaped grooves were introduced by single-point machining or rolling. Acetate replicas of the wheel surfaces taken after runs and samples of the as-cast strip were examined with a profilometer and compared.

### Example 1

### Thickness Variation

Qualitatively, it is easy to see the difference in strip quality using smooth and grooved wheels. Quantitatively, a definitive measure of strip quality is the thickness variation over a small area, for example one square inch, of the cast product due to defects. Measurements with flat and point micrometers were taken on samples cast on smooth wheels and those cast on grooved wheels according to the invention. The statistical difference between thickness measurements taken with flat micrometers and those with point micrometers weighted by the nominal thickness of the material (e.g. the percent difference) gives an indication of thickness variation over closely spaced regions. The similarly weighted difference between flat micrometer measurements and thickness calculated from the weight, length, width and density of the material gives a similar indication but without the subjective skill required to read a point micrometer. The results in Table 1 for 25.4 cm wide strip continuously cast on a clean, 71 cm diameter drum show that the thickness varies by twice as much over a small region of smooth-wheel-cast aluminum strip versus grooved-wheel-cast aluminum strip. Also, the scatter in the data (e.g., the "s" values) is much less for product cast on the grooved drums.

Where: N = number of casting experiments for which average thickness difference
statistics were evaluated. For each experiment, several individual samples were measured.
tₘ = average measured thickness variation, percent (point micrometer vs. flat micrometer) among N experiments
Sₘ = standard deviation, percent (among N experiments)
tₑ = average calculated thickness variation, percent (flat micrometer vs. calculated
from density)
Sₑ = standard deviation, percent (among N experiments).

Numerous (typically 10 to 20) sample measurements of thickness with flat and point micrometers were compiled to determine the average percent difference for strip from each of 21 separate strip casting trials on a smooth wheel representing different casting speed, pool, thickness, etc. These averages were then combined, resulting in an overall average, "At-m", with a variability defined as "Sₘ" for smooth-wheel casts.

Two separate grooves wheel strip casting experiments were evaluated in the above manner, and also by the similar (but easier) comparative method utilizing flat micrometer readings and "calculated thickness" values.

Table 1 shows:
a. A direct comparison between Δt̅ₘ and Sₘ for smooth and grooved wheels, and
b. the relationship between Δt̅ₘ and Δt̅_{c}, and between Sₘ and Sₑ for the same materials cast on a grooved wheel.

An additional 6 experiments on a grooved wheel were evaluated by the easier Δt̅_{c} method only. The results between the "group of 2" and the "group of 6" were statistically identical. By inference, we conclude that the "group of 2" and "group of 6" would have shown statistically identical Δt̅ₘ values if these had been determined for the "group of 6". This leads to the conclusion that the relative variability in thickness of product cast on "grooved" wheels is only about half of that for material cast on smooth wheels. The same conclusion results from Δt̅ₘ for only rows 1 and 2 of Table 1, but the added Δt̅_{c} values of row 3 make this conclusion much more certain.

### Example 2

Several trials were made using apparatus such as shown in Fig. 1 with a "smooth" wheel (i.e. a machined surface ground through 600-grit AI₂0₃ sanding paper then finished to a matte surface by peening with a rotating stainless steel brush). Aluminum 3105 alloy was melted and introduced to the chilled copper drum in a thin layer by the tundish. The drum surface was moving at between about 4 and 6 meters/second. A rotating wiper was used to keep the drum surface clean. A metallostatic head of about 4 inches was required to produce strip in a rather continuous mode. Strip quality varied, but dimples and other surface defects were plainly visible in virtually all the strip.

Trials with copper and steel on smooth drums produced similar defects in cast strip.

### Example 3

### Grooved Drum Casting

Additional trials were run using grooved drums. The drums were cleaned to remove any impurities, including any lubricants or other additive. Table 2 gives the conditions of each run. A brush was fixed to clean the wheel on each rotation after release of the strip.

The grooves appear to afford a preferred site (on the lands) for initiation of solidification and afford channels for escaping of entrained gases. Cast strip using the grooved drums showed substantially less defects on upper and lower surfaces than strip cast on smooth drums and substantially less thickness variability.

## Claims

1. Method for casting commercial quality metal sheet of thickness less than about 10 mm directly from the melt, comprising grooving the outer cylindrical surface of a chill wheel (2) with axially-spaced substantially circumferentially extending grooves (32) to produce a casting surface with a groove density of at least about 8 grooves per centimeter and rotating the chill wheel (2) and passing the grooved outer cylindrical surface through a melt pool (1) to extract a melt layer (10) onto the grooved outer surface, wherein the outer surface of this layer is unconfined and directly exposed to the atmosphere, characterised by providing substantially flat land regions (33) of at least 0.025 mm between adjacent grooves (32) and generally circumferential edges at the intersections of each land regions with the adjacent grooves, so that the adjacent surface of the melt layer directly contacts the land regions (33) and substantially spans the grooves (32) between land regions and withdrawing heat from the melt layer (10) through the grooved surface to progressively solidify the melt layer from the grooved surface to the melt layer outer surface.

2. Method of Claim 1 characterised by introducing the metal melt onto the outer surface having land regions (33) having a maximum width of 1.00 millimeter.

3. Method of Claim 2 characterised by introducing the metal melt onto the outer surface having a ratio of average groove (32) width to average land (33) width of between 0.5 and 1.5.

4. Method of Claim 2 characterised by introducing the metal melt onto the outer surface having a groove (32) depth of greater than about 0.025 millimeters.

5. Method of Claim 4 characterised in that the groove (32) depth is between about 0.025 and 0.25 millimeters.

6. Method of Claim 1 characterised by introducing the metal melt onto a peripheral surface of a drum (2) rotating at about 100-1000 cm/sec, wherein the grooves (32) are generally circumferential in the peripheral surface with a depth of about 0.025-0.25 millimeters and wherein the grooves are separated by land regions (33) having a width of less than about 0.635 millimeters.

## Patentansprüche

1. Verfahren zum Gießen von Metallbahnen kommerzieller Qualität mit einer Dicke von weniger als etwa 10 mm direkt aus der Schmelze, wobei die äußere, zylindrische Fläche eines Kühlrades (2) mit axial getrennten, im wesentlichen in Umfangsrichtung verlaufenden Nuten (32) genutet wird, um eine Gießfläche mit einer Nutendichte von wenigstens etwa acht Nuten pro cm gebildet wird, das Kühlrad (2) verdreht und die genutete, äußere, zylindrische Fläche durch ein Schmelzbad (1) geführt wird, um eine Schmelzschicht (10) auf der genuteten, äußeren Fläche zu extrahieren, wobei die äußere Fläche dieser Schicht unbegrenzt ist und direkt der Atmosphäre ausgesetzt ist, dadurch gekennzeichnet, daß im wesentlichen ebene Stegbereich (33) von wenigstens 0,025 mm zwischen benachbarten Nuten (32) und im wesentlichen, in Umfangsrichtung verlaufende Ränder an den Verschneidungen jedes Stegbereiches mit den benachbarten Nuten vorgesehen werden, so daß die benachbarte Fläche der Schmelzschicht direkt mit den Stegbereichen (33) in Kontakt steht und im wesentlichen die Nuten (32) zwischen Stegbereichen überspannt und Wärme von der Schmelzschicht (10) durch die genutete Fläche abzieht, um schrittweise die Schmelzschicht von der genuteten Fläche zur äußeren Fläche der Schmelzschicht zu verfestigen.

2. Verfahren nach Anspruch 1, dadurch gekennzeichnet, daß die Metallschmelze auf die äußere Fläche mit Stegbereichen (33) einer maximalen Breite von 1,00 mm aufgebracht wird.

3. Verfahren nach Anspruch 2, dadurch gekennzeichnet, daß die Metallschmelze auf die äußere Fläche mit einem Verhältnis der mittleren Breite der Nuten (32) zur mittleren Breite der Stege (33) von zwischen 0,5 und 1,5 aufgebracht wird.

4. Verfahren nach Anspruch 2, dadurch gekennzeichnet, daß die Metallschmelze auf die äußere Fläche mit einer Tiefe der Nuten (32) größer als etwa 0,025 mm aufgebracht wird.

5. Verfahren nach Anspruch 4, dadurch gekennzeichnet, daß die Tiefe der Nuten (32) zwischen etwa 0,025 und 0,25 mm ist.

6. Verfahren nach Anspruch 1, dadurch gekennzeichnet, daß die Metallschmelze auf die Umfangsfläche einer Trommel (2) aufgebracht wird, die bei etwa 100-1000 cm/s verdreht wird, wobei die Nuten (32) im wesentlichen in Umfangsrichtung auf der Umfangsfläche mit einer Tiefe von etwa 0,025 bis 0,25 mm sind und wobei die Nuten durch Stegbereiche (33) mit einer Breite von weniger als etwa 0,635 mm getrennt sind.

## Revendications

1. Procédé pour couler du métal en feuille de qualité commerciale, d'épaisseur inférieure à environ 10 mm, directement à partir du métal en fusion, selon lequel on rainure la surface cylindrique externe d'une roue de refroidissement (2) avec des rainures (32) s'étendant circonférenciellement espacées axialement de façon sensible pour former une surface de moulage avec une densité d'au moins 8 rainures par centimètre et on fait tourner la roue de refroidissement (2) et on fait passer la surface cylindrique rainurée extérieurement à travers un bain de métal en fusion, pour extraire une couche de métal en fusion (10) sur la surface externe rainurée, dans lequel la surface externe de cette couche n'est pas enfermée et est directement exposée à l'atmosphère, caractérisé en ce qu'on ménage des intervalles réallement plats (33) d'au moins 0,025 mm entre les rainures adjacentes (32) et des arêtes généralement circonférencielles aux intersections de chaque intervalle plat avec les rainures adjacentes, de sorte que la surface adjacente de la couche de métal en fusion touche directement les intervalles plats (33) et s'étend réellement au-dessus des rainures (32) entre les intervalles (33) et on enlève la chaleur de la couche de métal en fusion (10) à travers la surface rainurée pour solidifier progressivement la couche de métal en fusion de la surface rainurée jusqu'à la surface externe de la couche de métal en fusion.

2. Procédé selon la revendication 1, caractérisé en ce qu'on amène le métal en fusion sur la surface externe présentant les intervalles (33) avec une largeur maximum de 1 mm.

3. Procédé selon la revendication 2, caractérisé en ce qu'on amène le métal en fusion sur la surface externe présentant un rapport de largeur moyenne des rainures (32) à la largeur moyenne des intervalles (33) entre 0,5 et 1,5.

4. Procédé selon la revendication 2, caractérisé en ce qu'on amène le métal en fusion sur la surface externe présentant une profondeur de rainure supérieure à environ 0,025 mm.

5. Procédé selon la revendication 4, caractérisé en ce que la profondeur de rainure est entre environ 0,025 et 0,25 mm.

6. Procédé selon la revendication 1, caractérisé en ce qu'on introduit le métal en fusion sur une surface périphérique d'un tambour (2) tournant à environ 100-1000 cm/s, en ce que les rainures (32) sont généralement circonférencielles dans la surface périphérique avec une profondeur d'environ 0,025-0,25 mm et en ce que les rainures sont séparées par des intervalles (33) présentant une largeur inférieure à environ 0,635 mm.
